

## UNITED STATES PATENT OFFICE.

ROLAND LEIS, OF FRANCESVILLE, INDIANA.

## FURNITURE POLISH.

No Drawing.

Application filed August 14, 1923. Serial No. 657,432.

*To all whom it may concern:*

Be it known that I, ROLAND LEIS, a citizen of the United States, residing at Francesville, in the county of Pulaski and State of Indiana, have invented certain new and useful Improvements in Furniture Polish, of which the following is a specification.

This invention relates to an improved composition for polishing articles of furniture and the primary object of the invention is to provide an improved fluid which will not only effectively impart a high polish on the articles of furniture to which it is applied, but which will also form a tough and durable protecting skin therefor.

Another prime object of the invention is to provide an improved fluid for polishing furniture, which will effectively prevent the softening of the ordinary furniture finish and remove all scratches and scars therefrom.

Another object of the invention is to provide an improved polish embodying a coloring matter which will effectively stain any scratches in the polished surface of the furniture and thus prevent them from showing.

Another object of the invention is to provide a furniture polish which can be easily applied to the furniture and which will not become gummy in use.

With these and other objects in view, the invention consists in the combining of the following ingredients in the proportions named.

|                                |     |
|--------------------------------|-----|
| Pure raw linseed oil           | 72% |
| Pure turpentine                | 15% |
| Kerosene (coal oil)            | 10% |
| Castor oil                     | 2%  |
| Raw Turkey umber ground in oil | 1%  |

The ingredients are combined and mixed together in the ordinary manner common with paints or varnishes and the linseed oil acts as the vehicle as does the turpentine which also acts as a cleaning fluid. Kerosene acts as a filling and cleaning agent. The castor oil permits a high gloss to be obtained from the polish when the same is rubbed on the furniture. The raw Turkey umber acts as a coloring agent for the scratches and the like.

The furniture polish is preferably applied in a thin coat with a cloth on the article to be polished and then allowed to set from three to five minutes. It is then rubbed with a soft cloth to give it the gloss and finish. This will impart a high finish to the furniture and effectively remove all finger marks, scratches and the like therefrom and serve as a protecting coating for the ordinary finish.

From the foregoing description it can be seen that I have provided an improved furniture polish which acts as means for not only polishing the furniture but also as a means for protecting the ordinary finish of the furniture from harm.

Changes in details may be made without departing from the spirit or the scope of this invention.

What I claim as new is:—

A furniture polish comprising linseed oil 72%, pure turpentine 15%, kerosene 10%, castor oil 2%, and raw umber 1%.

In testimony whereof I affix my signature in presence of two witnesses.

ROLAND LEIS.

Witnesses:

HERBERT AMES,  
STANLEY SURBER.